

# UNITED STATES PATENT OFFICE.

LESLIE BRADFORD, OF BROKEN HILL, NEW SOUTH WALES, AUSTRALIA.

## SEPARATION OF METALLIC SULFIDS.

1,182,890.

Specification of Letters Patent. Patented May 16, 1916.

No Drawing.

Application filed September 10, 1913. Serial No. 789,017.

To all whom it may concern:

Be it known that I, LESLIE BRADFORD, subject of the King of Great Britain and Ireland, residing at Cummins street, Broken Hill, in the State of New South Wales, Commonwealth of Australia, have invented new and useful Improvements in the Separation of Metallic Sulfids, of which the following is a specification.

This invention relates to improvements in the separation of mixed sulfids more particularly to the separation of mixed lead and zinc sulfids, but it will be understood that I do not confine myself to the treatment of these mixed sulfids.

The object of this invention is to provide a process of effecting a preferential or selective separation by means of flotation of certain particles such as zinc sulfid (blende) or pyrites, or both, from sulfid particles of lead (galena) obtaining zinciferous or pyritic concentrates, or both, on the one hand and lead-containing concentrates on the other hand.

This invention is applied to the treatment of ores, concentrates, tailings, residues, slimes, and other products, and the term "ores" in this specification includes any mixture of metallic sulfids or metallic sulfids and gangue.

Hitherto flotation separation processes have only been generally applied to the general purpose of separating of the metallic sulfids from the gangue. Several different processes have been evolved for the separation of the zinc sulfids (blende) from the lead sulfids (galena) but these processes have been more or less dependent upon certain preliminary treatment or upon the conditions under which the separation is effected, and as a result thereof certain of the sulfids such as the lead sulfids (galena) are permanently affected upon their surface so that they are rendered more or less immune or insusceptible to flotation while the sulfids which have not been so affected are floated and produce the float concentrates.

According to my invention a preferential or selective flotation of the zinc sulfids (blende) or pyrites, or both, from the lead sulfids (galena) is effected by submitting the ores to flotation separation in a separating medium by which the lead sulfid particles (galena) are not chemically or otherwise permanently affected upon their sur-

face but by the action of the said medium itself the surfaces of the lead sulfid (galena) particles are brought into direct contact with the medium and the particles are "wetted" and thus temporarily rendered immune 60 or insusceptible to flotation while the other sulfids float. In contradistinction to the processes previously mentioned the lead sulfid particles (galena) are not permanently affected, that is to say that if the said particles 65 are subjected to a further flotation separation in the presence of a medium which does not of itself "wet" the surface of the said particles then they are susceptible to flotation and float concentrates may be obtained. 70

I find that a preferential flotation can be obtained of zinc sulfids (blende) or pyrites, or both, from lead sulfids (galena) by submitting the ores to flotation separation in 75 a medium comprising a solution (preferably a solution feebly acidulated) of one or more chlorids of the alkaline metals or alkaline earths.

I will now proceed to illustrate generally 80 the application of this invention. The ores or concentrates are ground to a state of fine division and slimed when found necessary to disassociate the different sulfid particles from each other and from the gangue. 85 The ground material is then submitted to a flotation separation (preferably an agitation or aeration flotation separation in which a frothing agent, such as oleic acid with heat is employed) in a medium consisting preferably of a solution of sodium chlorid acidulated with sulfuric acid or other commercial acid. In the treatment of mixed sulfid float concentrates which are the product of the ordinary acid flotation 90 treatments in the "wetting medium" (e. g. the saline solution) may be used in a neutral or alkaline condition in which case I find that the float concentrates usually require retreatment for the effective division of the 95 sulfid particles.

I prefer to have the flotation medium at a temperature ranging from 120° F. to 160° F. for I find that at this temperature the preferential separation of the zinc sulfid 105 (blende) or pyrites, or both, from the lead sulfid (galena) takes place most effectively but in some cases a preferential separation may be effected at lower temperatures and even at atmospheric temperature, but usu- 110

ally the float zinc concentrates produced at these lower temperatures require retreatment.

- The quantity of acid which is added to the wetting medium (e. g. saline solution) has an important bearing upon the preferential separation effected by this process. I am unable to indicate the degree of acidity required for all ores, but with certain ores with which I have experimented I find that if the acidity of the saline solution is increased to one per cent (1%) or thereabout the lead sulfid (galena) particles float more or less completely in addition to the zinc sulfid (blende) or pyrites, or both. I have found from experiments performed by me that a saline solution only feebly acidulated, that is containing 0.1 per cent. or 0.2 per cent. or thereabout is suitable for my purpose.
- If the process is applied directly to the preferential flotation of the zinc sulfids (blende) or pyrites, or both, from crude ores or the like containing lead sulfid and gangue the zinc sulfid (blende) and/or pyrites can if desired be separated without the addition of any organic frothing agent (such as oleic acid). The addition of a frothing agent may however be used without rendering the lead sulfid (galena) susceptible to flotation in the above described medium.

The quantity of saline substance in the preferential floating medium may be varied within wide limits. I find that a feebly acidulated solution containing about ten per cent. sodium chlorid well answers the purpose, but I do not bind myself to these directions.

- With regard to the nature of the saline salts employed I prefer to use common salt (sodium chlorid) owing to its cheapness. This flotation separation can be carried out in any well known apparatus in the ordinary way. I find then that a preferential flotation is effected inasmuch as the lead sulfid (galena) particles are temporarily "wetted" and thereby rendered non-susceptible to flotation in the aforesaid medium, and remain as a residue with the gangue, while the zinc sulfid (blende) or pyrites, or both, particles are not similarly affected and float, thereby producing a float concentrate comparatively high in zinc and low in lead.

In actual practice this invention may be applied in two different ways.

- In one application of the invention, the crude ores which have previously been crushed to a suitable state of division, may be submitted direct to the preferential flotation treatment herein described, producing float concentrates high in zinc, while the lead sulfid (galena) particles (being "wetted" by the special medium employed) remain with the gangue as a residue. Having thus preferentially removed the zinc sul-

fids (blende) the residues containing the major portion of the lead sulfids (galena) and the gangue are drained or washed, or both, for the removal of the "wetting medium" and submitted to a further flotation separation in the ordinary way by any of the well known methods producing a float concentrate high in lead.

In another application of the invention the crushed ore may be first of all subjected to a flotation separation in the ordinary way by any of the well known flotation methods (preferably that known as the "froth" flotation process in which the ore is agitated or aerated with a frothing agent (such as oleic acid) producing mixed concentrates without discrimination of the sulfids present. These mixed concentrates are then submitted to the special preferential flotation separation by agitating or aerating in the saline solution (preferably feebly acidulated) as aforesaid whereby the lead sulfid (galena) particles become "wetted" and are not susceptible to flotation in such medium, and are left as a high grade lead-containing residue on the one hand, while the zinc sulfids (blende) float producing a float concentrate high in zinc on the other hand.

In the treatment of an ore containing blende and galena with gangue, such as obtain at Broken Hill, New South Wales, I prefer to employ the second method above described. By applying the invention in this manner, both the floated zinc concentrates and the lead-containing residues are high grade marketable products and can be washed for the removal of the "wetting medium." A further advantage of this application of the invention is that the "wetting medium" is maintained in a greater state of purity than would be possible if the herein described preferential separation was applied direct to the crude ore. Lastly, the preferred method of applying the invention makes it possible to produce a cleaner and higher grade zinc concentrate.

In the case of ores, in a finely comminuted condition, as for example, mixed concentrates obtained in flotation processes using an organic frothing agent, I find that the division of zinc sulfid (blende) from lead sulfid (galena) by the aforesaid preferential flotation treatment is enhanced by first submitting the concentrates to a preliminary treatment with a grease-removing chemical for the purpose of removing any oil or oily substance or greasy hydrocarbon as by digestion in a dilute alkaline solution, e. g. in a dilute solution of sodium hydrate or carbonate or other alkaline hydrate or carbonate, or by treatment with a solution containing a small quantity of sulfuric ether. Further I find that with some ores more especially those in a finely comminuted

- condition—the zinc sulfids (blende) or pyrites, or both, agglomerate somewhat rapidly and have a tendency to mechanically include the lead sulfids (galena) in the flotation separation. It is desirable in these cases to add certain substances to the medium with the object of retarding the flotation effect on the zinc sulfids (blende) or pyrites, or both.
- 10 Substances which I find are suitable for the purpose are the lower sulfur acids and their salts such as the sulfites or thiosulfates of the alkaline metals or sulfurous acid. Solutions of these substances are added to the medium in sufficient quantity to produce the retardation desired enabling a cleaner separation of the zinc sulfids or pyrites, or both, from the lead sulfids. These substances must be added cautiously or the 15 flotation of the zinc sulfids (blende) or pyrites, or both, will be detrimentally affected. The ordinary metallurgical checks will sufficiently indicate the best working conditions.
- 20 I have not determined all the solutions which will form a suitable "wetting medium" for the purpose of my invention, but the same may be determined before operating or using my invention by the following 25 simple laboratory test:—Take 100 grams of the finely crushed ore; digest same in a dilute solution of caustic alkali, sulfuric ether or the like, then wash the ore. Both these steps are precautionary measures to 30 remove any deleterious constituents which may be present in the ore to be tested and which might interfere with the test. Transfer the ore to a glass cylinder (provided with a stopper) with a convenient amount 35 of boiling water; introduce the "wetting reagent" and agitate. Then add a small quantity of a ten per cent. solution of sulfuric acid and agitate. Test the liquor to ascertain whether it is acid or neutral by a drop 40 of methyl orange. If neutral add little more sulfuric acid (10 per cent. solution). Again agitate and test for acidity. Continue this operation until a faint permanent acidity is obtained. Then add a slight 45 excess of the ten per cent. solution of acid, sufficient to bring the medium up to say 0.1 per cent. or 0.2 per cent. strength. Add a small quantity of a "frothing agent" (such as oleic acid). Agitate violently for a sufficient length of time, and then critically inspect the contents of the cylinder. If the 50 "wetting reagent" employed in this particular test is found to leave the galena particles free and nongranulated, and at the same time permits the zinc sulfids (blende) particles or pyrites, or both, to granulate or coalesce together, it is an indication that the "wetting reagent" employed is suitable. If this test is made by the addition of a 55 minimum amount of "wetting reagent" and no differentiation between the zinc sulfids (blende) or pyrites, or both, and the lead sulfids (galena) is observable, repeat the test with a practical maximum quantity of the proposed "wetting reagent". In the description of the test above given stress has been laid on the quantity of sulfuric acid employed.
- 60 In submitting ores to the test I have found that if excessive amounts of acid are employed the galena particles are attacked by the acid and sulfureted hydrogen gas is evolved, and this gas if present in sufficient quantity and in the presence of the "frothing agent" causes a more or less partial 65 granulation of the galena particles and thus masks the test.
- To determine whether the wetting reagent is suitable for the purpose of this invention, and the quantity of same which will yield 70 the more effective result, and also the degree of heat required for different ores, actual flotation separation tests must be made by first floating the blende or pyrites, or both, with the employment of the "wetting medium" subsequently removing the remainder of the ore from the said medium, and floating the galena from same by the ordinary flotation methods, and assaying the 75 products in the usual manner.
- 80 What I claim is:—
1. A process for the preferential or selective separation of zinc sulfids from lead sulfids in ores containing mixed sulfids which consists in submitting the ores to agitation 85 with a frothing agent in a heated feebly acidulated solution of common salt of such a nature as to render the lead sulfid particles immune to flotation while in the said medium but as not to affect the subsequent 90 floatable properties of the said lead sulfid particles by the ordinary flotation treatments and which does not similarly affect the zinc sulfid particles and permits the said 95 zinc sulfid particles to float substantially in the manner hereinbefore described.
- 100 2. A process for the preferential or selective separation of zinc sulfids from lead sulfids in mixed sulfid concentrates obtained from an acid flotation separation which consists in submitting the said concentrates to agitation and aeration in a solution which does not chemically or otherwise permanently affect the lead sulfid particles upon 105 their surface but does by the action of the medium itself bring the surface of the lead sulfid particles into direct contact with the said medium and wets the said lead sulfid particles whereby the said lead sulfid particles sink and the zinc sulfid particles float 110 substantially in the manner hereinbefore described.
- 115 3. A process for the preferential or selective separation of zinc sulfids from lead sulfids in mixed sulfid concentrates obtained 120 from an acid flotation separation which consists in submitting the said concentrates to agitation and aeration in a solution which does not chemically or otherwise permanently affect the lead sulfid particles upon their surface but does by the action of the medium itself bring the surface of the lead sulfid particles into direct contact with the said medium and wets the said lead sulfid particles whereby the said lead sulfid particles sink and the zinc sulfid particles float 125 substantially in the manner hereinbefore described.
- 130

from an acid flotation separation which consists in submitting the said concentrates to agitation and aeration in a solution of a chlorid of such a strength as to preferentially wet said lead sulfids substantially in the manner hereinbefore described.

4. A process for the preferential or selective separation of zinc sulfids from lead sulfids in mixed sulfid concentrates obtained 10 from an acid flotation separation which consists in submitting the said concentrates to agitation and aeration in a heated solution of common salt of such a strength as to preferentially wet said lead sulfids obtaining float concentrates relatively high in zinc on the one hand and residues relatively high in lead on the other hand substantially in the manner hereinbefore described.

5. A process for the preferential or selective separation of zinc sulfids from lead sulfids in mixed sulfid concentrates obtained by any method of concentration which consists in submitting the said concentrates to agitation and aeration in a feebly acidulated 25 solution of common salt of such a strength as to preferentially wet said lead sulfids obtaining float concentrates relatively high in zinc on the one hand and residues relatively high in lead on the other hand substantially high in lead on the other hand substantially in the manner hereinbefore described.

30 6. A process for the preferential or se-

lective separation of zinc sulfids from lead sulfids in mixed sulfid concentrates obtained by any method of concentration which consists of submitting the said concentrates to agitation and aeration in a heated and feebly acidulated solution of common salt of such a strength as to preferentially wet said lead sulfids obtaining float concentrates relatively high in zinc on the one hand and residues relatively high in lead on the other hand substantially in the manner hereinbefore described.

7. A process for the preferential or selective separation of zinc sulfids from lead sulfids in mixed sulfids concentrates obtained by any method of concentration which consists in submitting the said concentrates to agitation and aeration in a feebly acidulated solution of common salt of such a strength as to preferentially wet said lead sulfids with the addition of an organic frothing agent obtaining float concentrates relatively high in zinc on the one hand and residues relatively high in lead on the other hand substantially in the manner hereinbefore described.

In testimony whereof I affix my signature in presence of two witnesses.

LESLIE BRADFORD.

Witnesses:

CHARLES STANLEY BURGESS,  
WINNIFRED WING.